

## UNITED STATES PATENT OFFICE

2,019,229

## COLORATION OF ALUMINUM ARTICLES

James Francis Leahy, Fairhaven, Mass., assignor  
to Atlas Tack Corporation, Fairhaven, Mass., a  
corporation of New York

No Drawing. Application November 16, 1931,  
Serial No. 575,459

5 Claims. (Cl. 148—6)

The subject of this invention is the coloration of aluminum objects and more particularly small aluminum articles, such as buttons, eyelets and the like. It has been found possible to effect a coloration of aluminum by using the aluminum base itself as a component entering into the chemical formation of the coloring material. More specifically it has been found that the superficial oxidation of aluminum articles to produce surface films or coatings of aluminum oxide on such articles, followed by the treatment of the articles with lake-forming dyes, results in the generation of insoluble color lakes tenaciously adherent to the aluminum base, the reaction evidently being analogous to that occurring when mordant dyes are fixed on textile goods with mordants of the class of aluminum oxide.

I have now discovered that if the oxide film formed on aluminum articles is brought to a predetermined condition of hydrogen ion concentration, more especially on the alkaline side of neutrality, it is possible to control and extend the tones of color or color effects and the appearance developed on the articles with the available lake-forming dyes. I have further found that by imparting a predetermined alkalinity to the aluminum oxide film, it is possible to ensure smooth and positive reaction between the film and the lake-forming dye to produce delicate and iridescent color lakes characterized by tenacious adherence to the metal base. The color effect obtained in any particular case depends upon the pH value or alkalinity of the solution to which the oxide film is exposed, and upon such other factors as time and temperature of treatment with the alkaline reagents.

While there are various ways of superficially oxidizing aluminum articles, I prefer to bring about such oxidation by a treatment such as disclosed in my application Serial Number 452,525, filed May 14, 1930. I shall therefore now give a specific example of procedure involving an initial oxidizing treatment of aluminum articles precisely as described in that application. Aluminum articles, such as buttons, are placed in a suitable perforated container or basket, and the basket then immersed in a solution of about 2% sodium carbonate and about ½% sodium bichromate, preferably at boiling temperature, as elevated temperature serves to accelerate the oxidizing reaction. The articles need remain in contact with the boiling solution for only five to fifteen minutes, at the end of which time a coating or skin of oxide of the desired depth has been produced and little further reaction takes place, probably owing to the impermeable character of the coating. The basket of articles is then removed from the solution and may be washed free of entrained solution, as by dipping in a bath of wash water. The oxide coating

formed on the articles is a mixture of both aluminum and chromium oxides, the sodium bichromate evidently being reduced by the metallic aluminum into an oxide while serving to oxidize the metallic aluminum into an oxide. The coating has a gray color characteristic of a mixture of both the aluminum and chromium oxides.

In accordance with the present invention, the batch of articles is then immersed in a solution of predetermined alkalinity, for instance, in a solution of both sodium carbonate and sodium tetraborate of about one tenth normality and in which the ratio of sodium carbonate to sodium tetraborate is about nine to one. The articles may be kept below the solution at about room temperature for about five minutes. The batch of articles may then be removed from the solution and subjected to the final dyeing operation. The alkaline treatment visibly modifies the oxide film, changing it from an opaque, dull-gray color to a condition of translucency or transparency. The thickness of the film is also reduced owing to the removal of considerable, if not all, of the chromium oxide as well as some of the aluminum oxide.

The dyeing of the articles may be performed in various lake-forming dye solutions. For instance, the batch of articles may be lowered into a bath of dye solution at about boiling temperature containing, for instance, 1% alizarin dye of the desired color, say, red, blue, green or a mixture of colors. The dye bath preferably contains about 1% of a weakly ionized acid such as formic, acetic, lactic, tartaric, boric or phosphoric; and the articles are permitted to remain in contact with the dye solution for about 15 minutes, at the end of which time practically equilibrium coloration has been effected. When alizarin sapphire is the dye employed the articles acquire an iridescent blue coloration, whereas, when alizarin orange is the dye employed, a delicate, gold-colored lake is fixed on the articles. The use of a dye bath at elevated temperature is highly desirable in that the reaction to form the colored coating or color lake is greatly accelerated by increase of temperature, comparatively little reaction taking place at room temperature. The colored articles may then be dried; and, if desired, this may be effected in a current of warm air, particularly inasmuch as no visible discoloration takes place under such conditions. The color lake formed on the article is resistant to scratching or abrasion and is characterized by its density, hardness and tenacity. It is firmly bonded with the aluminum base, although it can be removed by a hard, sharp instrument. The color lake also resists removal even by repeated treatment in solutions of alkali or soap, such as are used for laundering

purposes, so that aluminum buttons colored in accordance with my process are especially suitable for use on shirts or other articles of apparel which undergo repeated laundering treatment. In very considerable degree, the color lake is also resistant to fading or bleaching under the action of light.

The alkaline solution hereinbefore described for modifying the oxide film is subject to considerable variation in composition, depending upon the final color effect to be produced. Thus, the ratio of soda ash to borax in solution may be seven to three rather than nine to one, in which case the solution is less alkaline and accordingly reacts less drastically upon the oxide film. A solution containing borax alone, however, is incapable of accomplishing an observable modification of the oxide film when used at the normality or concentration specified in the foregoing example. In other words, as the concentration of sodium carbonate in solution is increased, there is a progressive increase in activity of the solution upon the film. Ordinarily it is preferable to keep the alkaline solution at relatively low chemical concentration, for instance at about one-tenth normality, so that flexibility or control of the reaction on the film may be had. The reaction may take place at room temperature, as indicated, but if desired the reaction may be hastened by heating the alkaline solution to about its boiling point. It is highly likely that under the conditions given in the cited example, the chromium oxide content of the film is practically entirely eliminated, since the color effects obtained are characteristic of those formed from aluminum oxide alone.

In practising the process of the present invention, it is essential that the solution employed for modifying the oxide film be of a particular hydrogen ion concentration on the alkaline side of neutrality, irrespective of the precise chemical relied upon to furnish the alkalinity. In this connection, it is to be observed that chemicals other than borax and/or sodium carbonate, for instance such salts as sodium phosphate, which hydrolyze in aqueous solution to yield solutions of relatively low alkalinity, may serve to cause the desired modification of the oxide film. This modification is, as already indicated, accompanied by chemical action of the alkaline solution upon the film. It is preferred to use alkaline solutions having a pH value falling between about ten, as the lower limit, and about eleven, as the upper limit. In actual commercial practice, alkaline solutions of a pH value of less than about ten are too slow in modifying the oxide film, whereas alkaline solutions having a pH value of greater than about eleven are too quick in their action on the film to permit easy control to the desired end-point of treatment.

I have adverted to the washing or rinsing of the preliminarily oxidized articles before they undergo the second alkaline treatment. The washing or rinsing step need not, however, be practised, since such little oxidizing solution as is entrained by the articles does not significantly modify the composition or action of the second alkaline solution. The articles may, however, undergo a succession of immersions, first, in the oxidizing bath, then in the alkaline bath, then in wash water, and finally in the dye bath. It is desirable, however, to maintain the oxide film in a wet or freshly formed state throughout the

process, since when the oxide film is once dried out, it does not react as desired with the dye solution unless it is rehydrated by special treatment. The entire process may be practised in a comparatively short period of time, at very low expense, and with little chemical consumption. The apparatus is of but the simplest kind; and a single container or basket serves for holding a batch of articles throughout the process. The process is one which, as already indicated, is amenable to accurate control, by which I mean that the finished product may be uniformly colored to the desired shade and that spoilage losses are averted. It is to be observed that although the initial treating solution may be slightly alkaline, it is nevertheless primarily an oxidizing agent, whereas the second treating solution is entirely free from oxidizing agents and serves primarily to exert a controlled alkaline reaction on the oxide film.

What I claim is:

1. A process which comprises treating aluminum articles with a solution of an oxidizing agent to form a coating of aluminum oxide thereon, then treating the articles with an alkaline solution whose pH value lies between about 10 and 11, and finally treating the articles with a lake-forming dye to generate an insoluble color lake on such articles.

2. A process of coloring small aluminum articles which comprises subjecting a batch of such articles to a succession of treatments, including a treatment with an oxidizing solution of sodium carbonate and sodium bichromate to form a coating of aluminum and chromium oxides on such articles, a treatment with a non-oxidizing alkaline solution whose pH value lies between about 10 and 11, and finally a treatment with a lake-forming dye solution to generate an insoluble color lake on such articles.

3. A process of coloring small aluminum articles which comprises subjecting a batch of such articles to a succession of treatments, including a treatment with an oxidizing solution of sodium carbonate and sodium bichromate to form a coating of aluminum and chromium oxides on such articles, a treatment with a mixed sodium tetraborate and sodium carbonate solution of about one-tenth normality and having a pH value lying between about 10 and 11, and finally a treatment with a lake-forming dye solution to generate an insoluble lake on such articles.

4. A process of coloring aluminum articles which comprises treating such articles with a solution of sodium carbonate and sodium bichromate to form a coating of aluminum and chromium oxides, while the coating is wet treating such articles with an alkaline solution whose pH value lies between about 10 and 11, and while the coating is still wet treating such articles with a solution of a lake-forming dye and a weakly ionized acid to generate an insoluble color lake on such articles.

5. A process which comprises treating aluminum articles with an oxidizing alkaline solution to form a coating of aluminum oxide thereon, then treating the articles with a non-oxidizing alkaline solution whose pH value lies between about 10 and 11, and finally treating the articles with a lake-forming dye to generate an insoluble color lake on such articles.